

## UNITED STATES PATENT OFFICE

JOSEPH A. KENNEDY, OF PAWTUCKET, RHODE ISLAND, ASSIGNOR TO ANACONDA WIRE  
AND CABLE COMPANY, OF NEW YORK, N. Y., A CORPORATION OF DELAWARE

METHOD OF TREATING PAPER WRAPPING STRIP

No Drawing.

Application filed May 19, 1930. Serial No. 453,717.

This invention relates to an improved method of preparing paper wrapping to be used in the manufacture of insulated cable and the like. In the manufacture of this cable, a paper strip is folded and wound spirally about the cable core to build up and form a protective covering therefor in lieu of the braid heretofore commonly used for such purpose. In this winding operation the paper strip passes through the folding die which in its contact with the edges of the strip is liable to break the edges thereof and interfere with the successful passage of the strip therethrough or even to tear the strip apart unless the edges are soft and pliable.

In preparing this strip for use the paper is rolled up and cut to form rolls of strip 1" wide and 10 $\frac{1}{4}$ " in diameter. Heretofore these rolls have been immersed in a bath of special wax to partially impregnate the paper therewith, after which they are placed in a closed receptacle and subjected to steaming. The steam melts the wax at the edges of the strip and these edges absorb moisture which acts to force the wax farther into the strip and relieve the stiffness of the paper and permit easy folding thereof. This treatment requires the use of a special high grade wax, which adds considerably to the expense of the treatment. It is the primary object of my invention to provide an improved and cheaper method of so treating these strip rolls with any wax, including the cheapest grade, that the edges of the strip are permanently rendered softer, more pliable and of a lubricated nature for smoother engagement with the die.

In accordance with my invention, I provide a wax bath, using any grade of wax, preferably a low priced grade for manufacturing economy, and immerse the rolls therein for a period of approximately ten minutes while keeping the bath at a temperature of about 260° F. This treatment saturates the paper with the wax through the entire roll. I then, preferably immediately, drop the rolls into a hot soap bath, i. e. hot water softened with soap. The soap which I have used and which I prefer to use in my improved process is commonly sold on the market and at the present time is known to the trade as "red oil fig soap". Other soaps might serve the purpose, but I have preferred this fig soap since it does not readily harden like common household soaps. This so-called "red oil fig soap" may be obtained in the open market. The so-called red oil fig soap comprises approximately 48% oleic acid, 7 $\frac{1}{2}$ % potassium hydroxide and has a water content ranging from 43% to 45%. In this treatment the soap permeates the wax and the edges of the strip and renders such edges softer and more pliable. The displacing of a large portion of the wax by the soap and the combining of the soap with a portion of the wax provides a lubricant on the edges of the strip, and this lubricant and the pliability of the edges are permanent, since the soap does not evaporate. The stiffness of and the strain on the paper is thus relieved and permits a smooth engagement of the strip edges with the die and the easy folding of the strip.

I am aware that attempts have been made heretofore to use a cheap wax for this process and that such attempts have not only failed but that the use of even the higher grades and more expensive waxes have been possible only when following the treatment with the steaming process heretofore referred to. My improved process not only permits the use of the cheapest grades of wax but considerably simplifies and cheapens the process by eliminating the steaming operation. Furthermore, my improved process produces an improved paper strip which is more pliable, more easily folded and with edges so permanently lubricated and smooth as to entirely eliminate any and all difficulties heretofore experienced in passing the strip through the folding die.

## I claim:

1. A method of processing rolls of paper strip to be used as wrapping in the manufacture of insulated conductors, consisting of treating the rolls in a bath of wax to saturate the paper, and thereafter treating the rolls in an aqueous soap solution to permeate and partially displace the wax with the soap at the

edges of the strip to render such edges soft and pliable.

2. A method of processing rolls of paper strip to be used as wrapping in the manufacture of insulated conductors, consisting of treating the rolls in a bath of wax to saturate the paper, and thereafter treating the rolls in an aqueous solution of non-hardening soap to permeate and partially displace the wax with the soap at the edges of the strip to render such edges soft and pliable.

3. A method of processing rolls of paper strip to be used as wrapping in the manufacture of insulated conductors, consisting of treating the rolls in a bath of wax to saturate the paper, and thereafter treating the rolls in a fig soap solution to permeate and partially displace the wax with the soap at the edges of the strip to render such edges soft and pliable.

4. A method of processing rolls of paper strip to be used as wrapping in the manufacture of insulated conductors, consisting of soaking the rolls in a hot wax bath to saturate the paper, and thereafter soaking the rolls in a hot solution of non-hardening soap to permeate and partially displace the wax with the soap at the edges of the strip.

5. A method of processing rolls of paper strip to be used as wrapping in the manufacture of insulated conductors, consisting of treating the rolls in a bath of wax to saturate the paper, and immediately thereafter placing the rolls in a hot soap solution to permeate and partially displace the wax with the soap at the edges of the strip to render such edges soft and pliable.

6. A method of processing rolls of paper strip to be used as wrapping in the manufacture of insulated conductors, consisting of treating the rolls for approximately ten minutes in a hot wax bath to saturate the paper, and thereafter treating the rolls in a fig soap solution including oleic acid and potassium hydroxide to permeate and partially displace the wax with the soap at the edges of the strip to render such edges soft and pliable.

7. A method of processing rolls of paper strip to be used as wrapping in the manufacture of insulated conductors, consisting of treating the rolls in a hot wax bath at a temperature of about 260°F. to saturate the paper, and thereafter treating the rolls in a soap solution to permeate and partially displace the wax with the soap at the edges of the strip to render such edges soft and pliable.

In testimony whereof I have affixed my signature..

JOSEPH A. KENNEDY.